

1

2,874,617

## METHOD OF DRYING WATER-LAID FIBROUS MATERIALS

Lewis W. Eckert, Lancaster Township, Lancaster County, Pa., assignor to Armstrong Cork Company, Lancaster, Pa., a corporation of Pennsylvania

No Drawing. Application June 30, 1955  
Serial No. 519,256

13 Claims. (Cl. 92—40)

This invention relates to a method of drying water-laid materials and is concerned more particularly with the drying of open, porous, fibrous materials subject to surface discoloration upon the application of heat above a limited temperature range.

This application is a continuation-in-part of my co-pending application, Serial No. 505,417, filed May 2, 1955, and entitled "Sound-Absorbing Unit and Method of Fabricating the Same."

In the manufacture of fibrous insulation products, such as wood fiberboard which is used for heat and sound insulation, the wood fibers are deposited onto a moving screen from a dilute slurry of the fibers in water. A small amount of flour or other binder may be incorporated into the furnish in some instances. The mass is consolidated to a desired thickness, water is removed by suction and pressure, and the dewatered web, still containing a large amount of water due to the porous nature of the product, is delivered to a drier where heat is applied to remove residual moisture. It has been found that, when drying fiberboards in a conventional flame heated drier, there is a tendency for the surface of the board to be discolored upon the application of relatively high temperatures to the surface of the board to facilitate the drying operation. As a consequence, the boards have been moved through the drier at a relatively slow speed and lower temperatures have been applied in order to effect the necessary drying of the product without discoloration. If it were possible to apply higher temperatures, the board could be moved through the drier faster and greater production could be achieved since the driers are the slowest unit in a conventional board-forming mill.

It is an object of the present invention to provide a method of drying which will permit the application of higher temperatures to the surface of fiberboards and the like without the disadvantage of objectionable discoloration of the surface.

While the discoloration problem is particularly acute in wood fiberboards, a similar problem exists in mineral fiber acoustical material fabrication where the product is made from mineral wool fibers dispersed in water and bound with starch or similar organic binding material. This product contains a large amount of water when delivered from the forming machine, and drying consequently is a major factor in the commercial production of the product. The product is disadvantageously discolored on the surface during drying at high temperatures, due probably to caramelizing or other degradation of the starch binder. The fibers themselves are not particularly susceptible to discoloration, since they are formed from mineral materials and are heat-resistant.

A further object of the invention is to provide a method of drying water-laid fibrous materials containing carbonaceous binders subject to discoloration, to permit the application of higher temperatures than normal to the surfaces of the product to dry them without objectionable discoloration resulting.

2

In the manufacture of wood fiber acoustical boards, there is some tendency for the surfaces of the boards to be of darker color than desired, due to the natural color of the fibers from which the board is produced. It is desirable, therefore, to effect a bleaching action on the fibers at the surface of the board if this can be done at a minimum of expense.

Another object of the invention is to provide a method of drying a wood fiberboard which will result in improvement in the surface color of the material, due to a bleaching action which is effected during drying at elevated temperatures.

According to the invention, there is applied to the surface of a formed body of felted fibers subject to heat discoloration, such as the wood fiber furnish or the starch and mineral wool fiber composition referred to above, while in wet condition and prior to drying, a solution of boric acid which penetrates into the body only slightly below the surface thereof. The fibrous mass is then passed into a drier, and water is removed. The boric acid serves to reduce discoloration of the product upon the application of temperatures which would normally result in objectionable discoloration; and it also serves, in some instances, to bleach the fibers and improve the surface color characteristics of the final dried product.

The invention first will be described in conjunction with the preparation of a wood fiber product.

A felted fibrous blank or body may be formed essentially from wood fibers. A wood fiberboard, prepared as 30 a water-laid web as disclosed in Scott Patent 2,642,359 is an example. The web may be formed on a conventional fiberboard-making machine, such as an Oliver forming machine, in which a slurry of fibers suspended in water is deposited upon a rotating screen and a continuous felted fibrous sheet is formed from which a portion of the water is extracted, the formed sheet being delivered over rolls to a press section, such as a Downingtown press, where additional water is removed from the sheet and it is consolidated to a desired thickness. The 40 formed sheet containing 65% to 75% by weight of water is delivered to a station where the upper surface of it in a wet condition has applied thereto a quantity of boric acid.

The boric acid is preferably in the form of an aqueous 45 solution. In order to assist in the control of the application of the solution to the wet board, particularly where the material is applied as a pool behind a metering roll, a thickening agent such as sodium alginate or the like may be combined with the boric acid solution.

In the preparation of a suitable treating material, the 50 following ingredients are combined, all parts being given by weight:

|                                            |       |
|--------------------------------------------|-------|
| Boric acid                                 | 8.00  |
| Sodium alginate (Keltex sold by Kelco Co.) | 0.25  |
| 55 Water                                   | 91.75 |

This provides an aqueous acid solution, the effective or active component of which consists essentially of boric acid.

In the preparation of the treating solution, the water 60 is heated to about 140° F., and the powdered sodium alginate is stirred in for about 5 to 15 minutes until a uniform distribution of it in the water has been obtained. Thereafter, the powdered boric acid is added, and the mixture is stirred for about 5 minutes. The solution is 65 maintained at a temperature of about 140° F. in order to insure that the boric acid will remain in solution. If a quantity of boric acid greater than about 8% is to be incorporated, then the temperature of the solution should be maintained at a higher level in order to insure complete solution of the boric acid in the water.

The boric acid in heated condition is applied to the

surface of the wet fiberboard sheet. Generally, a quantity equivalent to about 5 to 6 grams of boric acid on a dry weight basis is applied per square foot of surface of fiberboard treated and is adequate for the purposes of the present invention. However, larger quantities may be employed without deleterious results, and somewhat smaller quantities may be used.

At the time the boric acid treating solution is applied, the wet board as delivered from the Downingtown press may contain about 65% to 75% of water, as mentioned previously. The temperature of the board may be in the order of 100° F. The application of the heated boric acid solution to such a wet surface results in immediate interspersion of the boric acid treating solution and the water contained in the board, and a slight penetration of the boric acid solution into the body of the board occurs. It is desirable to limit the penetration to a very slight extent; and if too deep a penetration is obtained, the quantity of Keltex or other thickening agent may be increased.

The surface-treated board is then delivered to a drier. The first and middle zones may be heated to about 450° F. to 350° F. (from entrance to exit of each zone), and the exit zone may be similarly heated to about 370° F. to 260° F. It will be understood, of course, that until such time as substantially all of the water has been removed from the wet board the temperature of the board except at the outermost surface will not exceed about 212° F.; and in the inner areas, the board temperature will be much lower. At completion of the drying operation, however, the board at the upper treated surface may be elevated to a temperature in the order of 220° F. to 250° F. The board drying temperature and the duration of the drying time will vary with the thickness of the board; the quantity of water contained in the board at the time of delivery to the drier, the length of the drier zones, and other variable factors. In any event, the boric acid solution minimizes discoloration of the board surfaces and thus permits the use of higher drying temperatures than would otherwise be possible. Also, there is some bleaching action which occurs on the fibers through the application of the boric acid treating solution and its drying at elevated temperatures, and a lighter colored product is obtained than heretofore, using the same basic board-forming ingredients.

In another embodiment of the invention, a mineral wool sound-absorbing board furnish comprising nodulated mineral wool fibers 960 pounds, pearl starch and beater flour binder 165 pounds, wax size 13 pounds, and finely divided mineral filler 480 pounds, together with water sufficient to provide a total batch of about 960 gallons is formed into a sheet generally as disclosed in Alexander Patent 2,717,538 and, prior to fissuring of the product as disclosed in that patent, a coating of boric acid is applied to the upper surface of the board. In this embodiment, the boric acid solution, about 2.3% concentration, is applied at room temperature, about 70° F. to 90° F. The solution may be applied by spraying it onto the surface of the wet mass of formed mineral wool fibers and starch binder. It is a simple matter to control the quantity of applied solution with a liquid spray; and in this instance, no Keltex or other thickening agent is used, although if application by roll coater is desired or if too much penetration of the solution is obtained, a thickening agent may be added. With the starch bound mineral wool product referred to, about 2 grams of boric acid per square foot of board surface treated, on a dry weight basis, have been found adequate to minimize discoloration.

The treated board is delivered to a drier and drying is effected. It appears that the boric acid treatment renders the surface of the board less susceptible to discoloration due to the carmelizing or other degrading action of the starch binder which occurs; and as a result, higher temperatures than normal may be applied to the surface of the board without deleterious results. The temperature which may be tolerated without objectionable discolora-

tion will depend upon the nature of the carbonaceous binder, the quantity used in the product, the type of fibers used, and other variable factors. The boric acid treatment will in any event permit the attainment of higher

surface temperatures than would be possible without the boric acid at the surface. In practice with a mineral wool product containing a starch binder, temperatures as high as 675° F. to 700° F. in the initial zone and 400° F. to 450° F. in the final zone, with a measurable board surface temperature of about 400° F. at the instant of exit of the board from the drier, have been attained. The dried product exhibited less discoloration than the same boards without the boric acid coating dried at lower temperatures requiring a longer drying time.

15 The concentration of the boric acid solution which may be used may be varied as desired. Generally, a concentration of about 2% to 15% of boric acid in the treating solution will be found acceptable. With the lower concentrations, more solution must be applied to obtain 20 the desired quantity of boric acid for proper results, and the additional water must be removed from the board in the drier. If more concentrated solutions than 15% boric acid are used, then the temperature necessary to maintain the boric acid in solution may be objectionably high.

25 The total quantity of boric acid applied to the board may vary considerably; about 4 to 15 grams per square foot of surface of fiberboard of boric acid (on a dry weight basis) are adequate for most purposes with a 30 product such as the board of the Scott patent. With the mineral fiber acoustical material of the Alexander patent, where the fiber furnish is principally inorganic and the component subject to discoloration is in minor proportion, much less boric acid is required and as little as 1½ grams per square foot of board surface may be adequate. 35 The upper limit on the quantity of boric acid used is its cost and, where a water solution is used, the problem of saturation of the solution. Generally, about 15 grams per square foot of board surface are a good, practical maximum.

40 While sodium alginate is the preferred thickening agent, other thickening agents, such as carboxy methyl-cellulose and bentonite, may be substituted therefor, as is well known in the coating art. Generally, only a very 45 small quantity of thickening agent will be used, in the order of 0.25% to 1.0% of the total weight of the treating solution. Sufficient should be used to maintain most of the treating solution in the upper  $\frac{1}{16}$ " of the board. As noted in the mineral wool product example, the 50 thickening agent may be omitted.

55 While the invention has been described particularly in connection with the manufacture of insulating fiberboards and mineral wool acoustical units, it will be understood that the invention is applicable to all types of water-laid materials which are subject to discoloration upon the application of heat above a limited elevated temperature.

I claim:

60 1. In a method of drying a wet fibrous mass in board form to produce an open porous fibrous insulation board, the steps comprising applying directly to the upper surface of said wet fibrous board, in which the pores between the fibers are filled with water, 1.5 to 15 grams per square foot of surface on a dry weight basis of an aqueous acid solution, the effective component of which consists essentially of boric acid, to inhibit discoloration of 65 organic material which is contained in said board and which is subject to objectionable discoloration during drying, said application of the boric acid solution to the wet board resulting in interspersion of the boric acid solution with the water contained in the board and penetration of the boric acid solution into the body of the board below the upper surface thereof by diffusion into the water contained in the pores between the fibers of 70 the board; and thereafter drying said board by applying 75

heat thereto which elevates the surface temperature at said treated surface above the normal discoloration temperature of said organic material, a minimum temperature of 220° F., to form an open porous insulation board, said boric acid inhibiting said objectionable heat discoloration of said organic material at the treated surface of said board.

2. In a method of drying a wet fibrous mass in board form to produce an open porous fibrous insulation board, the steps of claim 1 in which the heat applied to the board is above 260° F.

3. In a method of drying a wet fibrous mass in board form to produce an open porous fibrous insulation board, the steps of claim 1 in which the fibrous mass comprises mineral wool fibers and an organic binder subject to objectionable discoloration during drying and in which heat applied to the board is in the range between 450° F. and 700° F.

4. In a method of drying a wet fibrous mass in board form to produce an open porous fibrous insulation board, the steps of claim 1 in which the fibrous mass comprises cellulosic fibers.

5. In a method of drying a wet fibrous mass in board form to produce an open porous fibrous insulation board, the steps of claim 4 in which the boric acid solution has incorporated therein a thickening agent which limits the penetration of the solution into about the upper  $\frac{1}{16}$ " of the board.

6. In a method of drying a wet fibrous mass in board form to produce an open porous fibrous insulation board, the steps of claim 4 in which the cellulosic fibers comprise wood fibers and in which an aqueous solution of boric acid is applied in an amount equivalent to about 4 to 15 grams dry weight per square foot of surface of the board treated.

7. In a method of drying a wet fibrous mass in board form to produce an open porous fibrous insulation board, the steps of claim 6 in which the board is dried at temperatures in the order of 450° to 260° F. from the beginning to the end of the drying cycle.

8. In a method of drying a wet fibrous mass in board form and including an organic binding material to produce an open porous fibrous insulation board, the steps comprising applying directly to the upper surface of said wet fibrous board, in which the pores between the fibers are filled with water, 1.5 to 15 grams per square foot of surface on a dry weight basis of an aqueous acid solution, the active component of which consists essen-

tially of boric acid, to inhibit discoloration of the organic binding material which is contained in said board and which is subject to objectionable discoloration during drying, said application of the boric acid solution to the wet board resulting in interspersion of the boric acid solution with the water contained in the board and penetration of the boric acid solution into the body of the board below the upper surface thereof through diffusion into the water contained in the pores between the fibers of the board, and thereafter drying said board by applying heat thereto which elevates the surface temperature at said treated surface above the normal discoloration temperature of said organic binding material, a minimum temperature of 220° F., to form an open porous insulation board, said boric acid inhibiting said objectionable heat discoloration of said organic binding material at the treated surface of said board.

9. In a method of drying a wet fibrous mass in board form to produce an open porous fibrous insulation board, the steps of claim 8 in which the organic binding material includes amylose material.

10. In a method of drying a wet fibrous mass in board form to produce an open porous fibrous insulation board, the steps of claim 8 in which the fibrous material comprises wood fibers.

11. In a method of drying a wet fibrous mass in board form to produce an open porous fibrous insulation board, the steps of claim 8 in which the fibrous material comprises mineral wool fibers.

12. In a method of drying a wet fibrous mass in board form to produce an open porous fibrous insulation board, the steps of claim 11 in which the board is exposed to temperatures in the order of 700° F. to 400° F. from the beginning to the end of the drying cycle.

13. In a method of drying a wet fibrous mass in board form to produce an open porous fibrous insulation board, the steps of claim 12 in which the organic binding material includes amylose material.

#### 40 References Cited in the file of this patent

#### UNITED STATES PATENTS

|           |            |                |
|-----------|------------|----------------|
| 1,153,970 | Sutherland | Sept. 21, 1915 |
| 1,738,976 | Vivas      | Dec. 10, 1929  |
| 1,784,566 | Andrews    | Dec. 9, 1930   |

#### FOREIGN PATENTS

|        |               |               |
|--------|---------------|---------------|
| 16,947 | Great Britain | Sept. 8, 1893 |
|--------|---------------|---------------|